

1

3,133,815

## COLOR PHOTOGRAPHIC MATERIALS AND PROCESSES

Colin William Greenhalgh, Manchester, England, assignor to Imperial Chemical Industries Limited, London, England, a company of Great Britain  
 No Drawing. Filed Aug. 29, 1960, Ser. No. 52,354  
 Claims priority, application Great Britain Mar. 20, 1957  
 14 Claims. (Cl. 96—55)

This application is a continuation-in-part of application Serial No. 716,857, filed February 24, 1958, and relates to materials and processes for color photography. Application Serial No. 52,353 filed concurrently herewith and being also a continuation-in-part of said application Serial No. 716,857 is concerned with the color couplers used in the materials and processes for color photography herein described, and with the manufacture of said color couplers.

In the practice of color photography dye images are produced by the reaction of the oxidation products of primary amino photographic developing agents, formed by the use of such developing agents in developing silver salt images, with certain classes of organic compounds which, as the result of such action, form azomethine, indophenol or related dyes. The developing agents used are usually N,N-dialkyl p-phenylene diamines or simple derivatives thereof, and the organic compounds which couple with the oxidation products of those developers, formed during development, are known as color couplers. These latter may contain amino groups and fall into several classes as follows:

(a) Those which contain, in addition to the amino group, a  $-\text{CO}-\text{CH}_2-\text{CO}-$  group. These normally yield yellow azomethine dyestuffs by coupling with the reaction products of, for example, N,N-diethyl p-phenylene diamine. Examples of such couplers are the compounds of the following formulae:



However, these are merely exemplary of a very large number of such compounds well known to the art.

(b) Those which contain, in addition to the amino group, a cyanoacetyl group or a pyrazolone ring. These normally yield magenta dyes by coupling as referred to

under (a). Examples of such couplers are the compounds of the following formulae:



Here again, the list given is merely exemplary of a very large number of such compounds well known to the art.

(c) Phenols or 1-naphthols which contain the amino group. These normally yield cyan dyes by coupling as referred to under (a). Examples of such couplers are the following:





This list is, of course, not exhaustive but purely exemplary, there being well known a very large number of such color couplers.

It is an object of the present invention to provide new materials for, and processes of, color photography which make use of derivatives of color couplers as aforesaid which have important advantages.

According to a first feature of the present invention there is provided a process for the production of a color photographic image which comprises subjecting a developable silver salt image to development by means of an aromatic primary amino color developing agent in the presence of a color coupler which in the form of its free acid is represented by the general formula:



where  $R-NH-$  represents the residue of a color coupler containing an amino group and either one of  $R_1$  and  $R_2$  is a hydrogen atom and the other is a group of the formula:



where  $R_3$  is a hydrogen atom or an alkyl, cycloalkyl, aralkyl or aryl radical and  $Z$  is an ethylene phenylene or tetrahydrophenylene radical.

More particularly according to the invention the said process is effected in the presence of a color coupler of the general formula:



where  $R-NH-$  is the residue of a color coupler containing an amino group selected from the class consisting of (a) color couplers which contain, in addition to the amino group, a  $-CO-CH_2-CO-$  group, (b) color couplers which contain, in addition to the amino group, a cyanacetyl group, (c) color couplers which contain in addition to the amino group a pyrazolone ring, and (d) colour couplers which contain the amino group and are phenols and 1-naphthols, and either one of  $R_1$  and  $R_2$  is a hydrogen atom and the other is a group of a structure selected from the group consisting of



where  $R_3$  is selected from the class consisting of a hydrogen atom, alkyl groups containing 1 to 18 carbon atoms, cycloalkyl groups containing 5 to 10 carbon atoms, aralkyl groups of which the alkyl moiety contains 1 to 3 carbon atoms, and aryl groups containing benzene and naphthalene ring systems, and  $Z$  is selected from the class consisting of ethylene, phenylene and tetrahydrophenylene radicals.

As examples of acyl groups there may be mentioned acetyl, propionyl, benzoyl, lauroyl, stearoyl, isobutyryl, caproyl, isovaleryl, ethylsulphonyl, hexadecylsulphonyl, and p-toluenesulphonyl.

As examples of alkyl groups represented by  $R_3$  there may be mentioned methyl, ethyl, butyl, heptyl, dodecyl, cetyl, octadecyl, iso-butyl, iso-amyl and tert-octyl.

As examples of cycloalkyl groups represented by  $R_3$  there may be mentioned cyclopentyl, cyclohexyl, hexahydrobenzyl and cyclodecyl.

As examples of aralkyl groups represented by  $R_3$  there may be mentioned benzyl, p-dodecylbenzyl,  $\beta$  benzyl-isopropyl, naphthyl methyl, phenyl ethyl and phenyl propyl, and as examples of aryl groups represented by  $R_3$  there may be mentioned phenyl, tolyl, chlorophenyl, sulphonophenyl, methoxyphenyl cyanophenyl, naphthyl and dodecylphenyl.

The symbol  $R-NH-$  may represent the residue of any of the specific amino color couplers which are listed above (i.e. the residue obtained by removing a hydrogen atom from the amino group), or the residue of any other amino color coupler within the generic groupings specified above. It is particularly to be noted that the nature of the amino color coupler residue is not critical. Any of the types known in this art may be used. The critical feature in the applicant's products is the chain



referred to above which characterises the products and leads to the advantages referred to above. Nevertheless, from the standpoint of color photography in natural colors it is obviously desirable to select the amino color coupler used as starting material so that the color coupler according to the present invention is of satisfactory hue, i.e. in one of the subtractive colors, yellow, magenta and cyan.

The aforesaid color couplers wherein  $R_1$  or  $R_2$  stands for  $-N\text{-}R_3\text{-acyl}$ , may be prepared by reacting a color coupler containing an amino group with an anhydride of the formula:



wherein  $R_3$  has the meaning stated above.

The reaction between the color coupler containing an amino group and the anhydride may be conveniently carried out by heating the reactants together in a suitable organic solvent, for example glacial acetic acid.

The new color couplers may be conveniently isolated by adding water and/or an aliphatic alcohol, for example methanol and ethanol to the solution of the color coupler in the organic solvent and filtering off the solid which is precipitated.

The color coupler so obtained consists of either or both of the two isomeric compounds which are obtainable by reacting the color coupler containing an amino group with an anhydride of the above formula.

The anhydrides of the above formula may be obtained by heating an amino acid of the formula:



wherein  $R_3$  has the meaning stated above with an acid chloride or an acid anhydride.

The amino acids of the above formula may themselves be obtained by treating maleic acid with ammonia, or an alkylamine or a cycloalkylamine or an aralkylamine or an arylamine.

Alternatively the anhydride of the above formula may be obtained by reacting an ester of maleic acid with ammonia, or an alkylamine, or a cycloalkylamine, or an aralkylamine or an arylamine, subsequently treating with an acid chloride or an acid anhydride, hydrolysing off the ester groups and subsequently treating with a dehydrating agent, for example acetic anhydride.

As examples of suitable anhydrides which may be used in this process of the invention there may be mentioned stearoylaminosuccinic anhydride, acetylaminosuccinic anhydride, lauroylaminosuccinic anhydride, benzoylaminosuccinic anhydride, N-benzylacetylaminosuccinic anhydride, phenylacetylaminosuccinic anhydride, butyl-isobutyrylaminosuccinic anhydride, N-cetylacetylaminosuccinic anhydride, N-n-octadecylacetylaminosuccinic anhydride, N-n-octadecylpropionylaminosuccinic anhydride, N-n-octadecyl-iso-butyrylaminosuccinic anhydride, N-n-octadecyl-isovalerylaminosuccinic anhydride, N-n-hexadecylbenzoylaminosuccinic anhydride, N-n-butylacetylaminosuccinic anhydride, N-p-dodecyl-p-benzylacetylaminosuccinic anhydride, N-p-dodecylphenyl-iso-butyrylaminosuccinic anhydride, p-toluenesulphonylaminosuccinic anhydride, n-hexadecylsulphonylaminosuccinic anhydride and N-p-dodecylphenyl-propionylaminosuccinic anhydride.

The new color couplers wherein  $R_1$  or  $R_2$  stands for



may be prepared by reacting a color coupler containing an amino group with a compound of the formula:



where  $Z$  has the meaning stated above.

The reaction between the color coupler containing the amino group and the compound of the above formula may be conveniently carried out by heating the reactants together in a suitable organic solvent, for example glacial acetic acid, and subsequently precipitating the new color coupler by the addition of water and/or methanol and ethanol.

The color coupler so obtained consists of either or both of the two isomeric compounds which are obtainable by reacting the color coupler containing an amino group with a compound of the above formula.

The compounds of the above formula may themselves be obtained by reacting aminosuccinic acid with an anhydride of an ethylene, phenylene or tetrahydrophenylene dicarboxylic acid, and subsequently treating with a dehydrating agent, for example acetic anhydride.

As examples of suitable compounds of the above formula which may be used in this process of the invention there may be mentioned phthalimidosuccinic anhydride.

5 The color couplers containing an amino group which may be used in the production of the color couplers for use in the present invention are, for example, those listed above.

Sixty-four specific examples of color couplers for use in the present invention, together with their method of preparation, are set out in co-pending application Serial No. 52,353 referred to above. They are:

- 10 1-phenyl-3-( $\beta$ -stearoylamino- $\beta$ -carboxypropionylamino)-5-pyrazolone,
- 15 1-phenyl-3-( $\alpha$ -stearoylamino- $\beta$ -carboxypropionylamino)-5-pyrazolone,
- 20 1-phenyl-3-[4'-( $\beta$ -stearoylamino- $\beta$ -carboxylpropionylamino)-phenoxyacetylamino]-5-pyrazolone,
- 25 1-phenyl-3-[4'-( $\alpha$ -stearoylamino- $\beta$ -carboxypropionylamino)-phenoxyacetylamino]-5-pyrazolone,
- 30 1-phenyl-3-[4'-( $\beta$ -stearoylamino- $\beta$ -carboxypropionylamino)-benzylamino]-5-pyrazolone,
- 35 1-phenyl-3-[4'-( $\alpha$ -stearoylamino- $\beta$ -carboxypropionylamino)-benzylamino]-5-pyrazolone,
- 40 4- $\omega$ -cyanoacetyl-( $\beta$ -stearoylamino- $\beta$ -carboxypropionylamino),
- 45 4- $\omega$ -cyanoacetyl-( $\alpha$ -stearoylamino- $\beta$ -carboxypropionylamino),
- 50 1-hydroxy-2-naphtho-N-( $\beta$ -stearoylamino- $\beta$ -carboxypropionylamino)-ethylamide,
- 55 1-hydroxy-2-naphtho-N-( $\alpha$ -stearoylamino- $\beta$ -carboxypropionylamino)-ethylamide,
- 60 4'-methoxybenzoylacet-4-( $\beta$ -stearoylamino- $\beta$ -carboxypropionylamino)-2-methoxyanilide,
- 65 4'-methoxybenzoylacet-4-( $\alpha$ -stearoylamino- $\beta$ -carboxypropionylamino)-2-methoxyanilide,
- 70 5-( $\beta$ -stearoylamino- $\beta$ -carboxypropionylamino)-1-naphthol,
- 75 5-( $\alpha$ -stearoylamino- $\beta$ -carboxypropionylamino)-1-naphthol,
- 80 4'-methoxybenzoylacet-5-{ $\beta$ -[N-(4-n-dodecylphenyl)propionylamino]- $\beta$ -carboxypropionylamino}-2-methoxyanilide,
- 85 4'-methoxybenzoylacet-5-{ $\alpha$ -[N-(4-n-dodecylphenyl)propionylamino]- $\beta$ -carboxypropionylamino}-2-methoxyanilide,
- 90 4'-methoxybenzoylacet-5-{ $\beta$ -[N-(4-n-dodecylphenyl)isobutyrylamino]- $\beta$ -carboxypropionylamino}-2-methoxyanilide,
- 95 4'-methoxybenzoylacet-5-{ $\alpha$ -[N-(4-n-dodecylphenyl)isobutyrylamino]- $\beta$ -carboxypropionylamino}-2-methoxyanilide,

amino)- $\beta$ -carboxypropionylamino]-2-methoxyanilide,  
 4'-methoxybenzoylacet-5-[ $\beta$ -(N-n-octadecylisobutyryl-  
 amino)- $\beta$ -carboxypropionylamino]-2-diethylamino-  
 anilide,  
 4'-methoxybenzoylacet-5-[ $\alpha$ -(N-n-octadecylisobutyryl-  
 amino)- $\beta$ -carboxypropionylamino]-2-diethylamino-  
 anilide,  
 4'-methoxybenzoylacet-5-[ $\beta$ -(N-n-octadecylacetyl-  
 amino)- $\beta$ -carboxypropionylamino]-2-methoxyanilide,  
 4'-methoxybenzoylacet-5-[ $\alpha$ -(N-n-octadecylacetyl-  
 amino)- $\beta$ -carboxypropionylamino]-2-methoxyanilide,  
 4'-methoxybenzoylacet-5[ $\beta$ -(N-(4-n-dodecylphenyl)-  
 acetylamino] $\beta$ -carboxypropionylamino]2-methoxy-  
 anilide,  
 4'-methoxybenzoylacet-5[ $\alpha$ -(N(4-n-dodecylphenyl)-  
 acetylamino] $\beta$ -carboxypropionylamino]2-methoxy-  
 anilide,  
 4'-methoxybenzoylacet-4[ $\beta$ -(N-n-butylacetyl-  
 amino)- $\beta$ -carboxypropionylamino]-2-methoxyanilide,  
 4'-methoxybenzoylacet-4[ $\alpha$ -(N-n-butylacetyl-  
 amino)- $\beta$ -carboxypropionylamino]-2-methoxyanilide,  
 4'-methoxybenzoylacet-5( $\beta$ -benzoylamino- $\beta$ -carboxy-  
 propionylamino)-2-methoxyanilide,  
 4'-methoxybenzoylacet-5( $\alpha$ -benzoylamino- $\beta$ -carboxy-  
 propionylamino)-2-methoxyanilide,  
 4'-methoxybenzoylacet-5( $\beta$ -benzoylamino- $\beta$ -carboxy-  
 propionylamino)-2-diethylaminoanilide,  
 4'-methoxybenzoylacet-5( $\alpha$ -benzoylamino- $\beta$ -carboxy-  
 propionylamino)-2-diethylaminoanilide,  
 4'-methoxybenzoylacet-2-( $\beta$ -stearoylamino- $\beta$ -carboxy-  
 propionylamino)-4-methoxyanilide,  
 4'-methoxybenzoylacet-2-( $\alpha$ -stearoylamino- $\beta$ -carboxy-  
 propionylamino)-4-methoxyanilide,  
 2'-methyl-2':3'-dihydrobenzofuran-7'-ylcarbonylacet-4-( $\beta$ -  
 stearoylamino- $\beta$ -carboxypropionylamino)-2-methoxy-  
 anilide,  
 2'-methyl-2':3'-dihydrobenzofuran-7'-ylcarbonylacet-4-( $\alpha$ -  
 stearoylamino- $\beta$ -carboxypropionylamino)-2-methoxy-  
 anilide,  
 4'-methoxybenzoylacet-5-[ $\beta$ -(N-n-octadecylisobutyryl-  
 amino)- $\beta$ -carboxypropionylamino]-2-methoxyanilide,  
 4'-methoxybenzoylacet-5-[ $\alpha$ -(N-n-octadecylisobutyryl-  
 amino)- $\beta$ -carboxypropionylamino]-2-methoxyanilide,  
 2-[3-[ $\beta$ -(N-i-octadecylisobutyryl-  
 amino)- $\beta$ -carboxypropionylamino]- $\beta$ -carboxypro-  
 pionylamino]-benzoylamino]-4-chloro-5-methylphenol,  
 2-[3-[ $\alpha$ -(N-n-octadecylisobutyryl-  
 amino)- $\beta$ -carboxypropionylamino]- $\beta$ -carboxypro-  
 pionylamino]-benzoylamino]-4-chloro-5-methylphenol,  
 1-hydroxy-4-chloro-2-naphtho-N-[3-[ $\beta$ -(N-n-octadecyl-  
 isobutyryl-  
 amino)- $\beta$ -carboxypropionylamino]-benzyl-  
 amino]-amide,  
 1-hydroxy-4-chloro-2-naphtho-N-[3-( $\beta$ -stearoylamino- $\beta$ -  
 carboxypropionylamino)-benzylamino]-amide,  
 1-hydroxy-4-chloro-2-naphtho-N-[3-( $\alpha$ -stearoylamino- $\beta$ -  
 carboxypropionylamino)-benzylamino]-amide,  
 1-hydroxy-4-chloro-2-naphtho-N-[ $\beta$ ( $\beta$ -stearoylamino- $\beta$ -  
 carboxypropionylamino)-ethyl]amide,  
 1-hydroxy-4-chloro-2-naphtho-N-[ $\beta$ ( $\alpha$ -stearoylamino- $\beta$ -  
 carboxypropionylamino)ethyl]amide,  
 2[ $\beta$ -(N-n-octadecylisobutyryl-  
 amino)- $\beta$ -carboxypropionyl-  
 amino]-4:6-dichloro-5-methylphenol,  
 2[ $\alpha$ -(N-n-octadecylisobutyryl-  
 amino)- $\beta$ -carboxypropionyl-  
 amino]-4:6-dichloro-5-methylphenol,  
 2( $\beta$ -stearoylamino- $\beta$ -carboxypropionylamino)4:6-di-  
 chloro-5-methylphenol,  
 2( $\alpha$ -stearoylamino- $\beta$ -carboxypropionylamino)-4:6-di-  
 chloro-5-methylphenol,  
 2( $\beta$ -stearoylamino- $\beta$ -carboxypropionylamino)-6-methyl-  
 phenol,  
 2( $\alpha$ -stearoylamino- $\beta$ -carboxypropionylamino)-6-methyl-  
 phenol,  
 2( $\beta$ -stearoylamino- $\beta$ -carboxypropionylamino)-5-chloro-  
 phenol,

2( $\alpha$ -stearoylamino- $\beta$ -carboxypropionylamino)-5-chloro-  
 phenol,  
 3( $\beta$ -stearoylamino- $\beta$ -carboxypropionylamino)phenol,  
 3( $\alpha$ -stearoylamino- $\beta$ -carboxypropionylamino)phenol,  
 5 2[ $\beta$ -(N-n-octadecylisobutyryl-  
 amino)- $\beta$ -carboxypropionyl-  
 amino]-4-chloro-5-methylphenol,  
 2[ $\alpha$ -(N-n-octadecylisobutyryl-  
 amino)- $\beta$ -carboxypropionyl-  
 amino]-4-chloro-5-methylphenol,  
 2( $\beta$ -stearoylamino- $\beta$ -carboxypropionylamino)-5-meth-  
 oxyphenol,  
 2-( $\alpha$ -stearoylamino- $\beta$ -carboxypropionylamino)-5-meth-  
 oxyphenol,  
 1-hydroxy-2-naphtho-N{ $\beta$ [ $\beta$ -(N-n-octadecylpropionyl-  
 amino)- $\beta$ -carboxypropionylamino]ethyl}amide,  
 15 1-hydroxy-2-naphtho-N{ $\beta$ [ $\alpha$ -(N-n-octadecylpropionyl-  
 amino)- $\beta$ -carboxypropionylamino]-ethyl}amide,  
 1-hydroxy-2-naphtho-N-[ $\beta$ -[ $\beta$ -(N-4-n-dodecylphenyl)-  
 propionylamino- $\beta$ -carboxypropionylamino]ethyl}amide,  
 20 1-hydroxy-2-naphtho-4-[ $\beta$ -[ $\alpha$ -(N-4-n-dodecylphenyl)-  
 propionylamino- $\beta$ -carboxypropionylamino]ethyl}amide,  
 1-hydroxy-4-chloro-2-naphtho-N{ $\beta$ -[ $\beta$ -(N-n-octadecyl-  
 isobutyryl-  
 amino)- $\beta$ -carboxypropionylamino]ethyl}amide,  
 25 1-hydroxy-4-chloro-2-naphtho-N{ $\beta$ -[ $\alpha$ -(N-n-octadecyl-  
 isobutyryl-  
 amino)- $\beta$ -carboxypropionylamino]ethyl}amide,  
 4- $\omega$ -cyanoacetyl-[ $\beta$ -(4-n-dodecylphenyl)acetyl-  
 amide,  
 4- $\omega$ -cyanoacetyl[ $\alpha$ -(4-n-dodecylphenyl)acetyl-  
 amide,  
 1-phenyl-3-[ $\beta$ -(N-n-butylisobutyryl-  
 amino)- $\beta$ -carboxypropionylamino]-5-pyrazolone,  
 30 1-phenyl-3-[ $\alpha$ -(N-n-butylisobutyryl-  
 amino)- $\beta$ -carboxypropionylamino]-5-pyrazolone.

The aforesaid color couplers may be used in the photographic developing solution used for developing a photographic emulsion, or they may be included in the photographic material, in a light-sensitive layer or in a non-light-sensitive layer adjacent to a sensitive layer or separated therefrom by a water-permeable colloid layer.

It is a preferred feature of the invention to include the aforesaid color couplers in a light-sensitive gelatinous or gelatino-substitute silver halide emulsion layer which forms part of a multi-layer film or paper of the kind used for color photography. For this purpose it is preferred to use those new color couplers which contain a substituent rendering them fast to diffusion, for example an alkyl chain containing at least 12 carbon atoms. If desired the new color couplers may be used in the form of their salts with an alkali metal or an organic amine.

The multilayer photographic material may be a natural order material in which the images are to be formed in colors complementary to those of the original object or one in which an unnatural order is used, for example one in which in the top layer there is formed a yellow image of the blue parts of the object, in one of the two lower layers there is formed a cyan image of the green parts of the object and in the other a magenta image of the red parts of the object.

The color couplers used in the present invention have important advantages over the color couplers from which they are derived. In particular it has been found that when a light-sensitive gelatinous or gelatino-substitute silver halide emulsion layer containing an aforesaid color coupler is exposed to light, developed in a color-forming developer, bleached and fixed, and the photographic record so formed is exposed to light, there is little or no staining of the record due to degradation by light of unreacted color coupler residual in the layer containing the dyestuff image.

The invention is illustrated, but not limited, by the following examples in which the parts and percentages are by weight:

**9**  
**EXAMPLES**

The color couplers used have the general formula:



where A=color coupling residue and R<sub>1</sub> or R<sub>2</sub> is H and the other is



where R<sub>3</sub>=H, alkyl, cycloalkyl, aralkyl, or aryl and Z is an ethylene, phenylene or tetrahydro phenylene radical.

The color formers are obtained by the reaction of A-NH<sub>2</sub> with either



where A, R<sub>3</sub> and Z have the meanings given above.

The color couplers are formulated in a photographic emulsion layer according to one of the following methods.

(I) To 200 parts of a green-sensitive gelatino-silver iodobromide emulsion there are added 50 parts of a 5% aqueous or aqueous methanolic solution of the potassium or other alkali metal salt of the color coupler. Alternatively an equivalent amount of an aqueous dispersion of the color coupler, obtained by standard dispersion techniques in the presence of a suitable dispersing agent as, for example, diethyl sulfo succinate, may be used. The emulsion so obtained is coated on a film or paper base

**10**

and the coated layer is dried. When the photographic layer is exposed to green light, developed in a color developer solution containing a color developing agent, which for example may be 4-amino-3-methyl-N-diethylaniline (B), 4-amino-3-methyl-N-ethyl-N- $\omega$ -hydroxybutyl aniline (C) or 4-amino-N-ethyl-N-hydroxyphenyl aniline (D), bleached and fixed, a magenta dye image is obtained.

(II) In place of the 200 parts of green-sensitive gelatino-silver iodobromide emulsion used in (I), there are used 10 200 parts of a blue-sensitive gelatino-silver iodobromide emulsion. When the coated layer is exposed to blue light and processed as described under (I), a yellow dye image is obtained.

(III) In place of the 200 parts of green-sensitive silver iodobromide emulsion used in I there are used 200 parts of a red-sensitive iodobromide emulsion. When the coated layer is exposed to red light and processed as described under (I), a cyan dye image is obtained.

(IV) When the color coupler does not contain a long 20 aliphatic chain it may be incorporated in a color developer solution, for example:

80 parts of trisodium phosphate and 1.2 parts of hydroxylamine sulphate are dissolved in 400 parts of water (solution A). 2 parts of the color coupler are dissolved 25 (or suspended) in 100 parts of ethanol (B). 2 parts of the color developing agent, 10 parts of anhydrous sodium sulphite and 4 parts of potassium bromide are dissolved in 400 parts of water (solution C). B is added to solution A, solution C then being added with stirring 30 and the volume made up to 1000 parts with water.

When a film carrying a gelatino-silver halide emulsion is exposed and then developed in the developer solution and subsequently bleached and fixed, a dye image is obtained.

| Example No. | Structure of color coupler R-NHCOCH(R <sub>1</sub> )-CH(R <sub>2</sub> )-COOH |                                                                                                                           | Formulation Process | Developing Agent | $\lambda_{max}$ |
|-------------|-------------------------------------------------------------------------------|---------------------------------------------------------------------------------------------------------------------------|---------------------|------------------|-----------------|
|             | R                                                                             | R <sub>1</sub> or R <sub>2</sub> where one is H                                                                           |                     |                  |                 |
| 1           |                                                                               | -NHCOC <sub>17</sub> H <sub>35</sub>                                                                                      | I                   | B                | 536             |
| 2           |                                                                               | -NHCOC <sub>17</sub> H <sub>35</sub>                                                                                      | I                   | B                | 540             |
| 3           |                                                                               | -NHCOC <sub>17</sub> H <sub>35</sub>                                                                                      | I                   | B                | 519             |
| 4           |                                                                               | -NHCOCH <sub>2</sub> O-C <sub>2</sub> H <sub>5</sub> OOC-C <sub>6</sub> H <sub>4</sub> -N=N-C <sub>6</sub> H <sub>5</sub> | I                   | {B<br>C}         | 532<br>534      |
| 5           |                                                                               | -NHCOCH <sub>2</sub> O-C <sub>6</sub> H <sub>4</sub> -Cl                                                                  | I                   | {B<br>C}         | 533<br>529      |
| 6           |                                                                               | -N(C <sub>18</sub> H <sub>37</sub> )COCH <sub>3</sub>                                                                     | I                   | {B<br>C}         | 528<br>536      |
| 7           |                                                                               | -N(C <sub>18</sub> H <sub>37</sub> )COCH <sub>3</sub>                                                                     | I                   | {B<br>C}         | 532<br>535      |

| Example No. | Structure of color coupler R—NHCOCH <sub>2</sub> —CH <sub>2</sub> —COOH |                                                                                                                | Formulation Process | Developing Agent | λ max.            |
|-------------|-------------------------------------------------------------------------|----------------------------------------------------------------------------------------------------------------|---------------------|------------------|-------------------|
|             | R                                                                       | R <sub>1</sub> R <sub>2</sub>                                                                                  |                     |                  |                   |
| 8           |                                                                         | —N—<br>nC <sub>18</sub> H <sub>37</sub><br>COCH <sub>3</sub>                                                   | I                   | {B<br>C          | 532<br>535        |
| 9           |                                                                         | —N—<br>nC <sub>18</sub> H <sub>37</sub><br>COCH(CH <sub>3</sub> ) <sub>2</sub>                                 | I                   | {B<br>C          | 526<br>533        |
| 10          |                                                                         | —N—<br>nC <sub>18</sub> H <sub>37</sub><br>COCH(CH <sub>3</sub> ) <sub>2</sub>                                 | I                   | {B<br>C          | 531<br>534        |
| 11          |                                                                         | —N—<br>nC <sub>18</sub> H <sub>37</sub><br>COCH <sub>2</sub> CH <sub>2</sub> CH(CH <sub>3</sub> ) <sub>2</sub> | I                   | {B<br>C<br>D     | 530<br>538<br>526 |
| 12          |                                                                         | —NHSO <sub>2</sub> C <sub>6</sub> H <sub>5</sub>                                                               | I                   | {B<br>C<br>D     | 531<br>539<br>525 |
| 13          |                                                                         | —NHSO <sub>2</sub> C <sub>6</sub> H <sub>4</sub> Cl                                                            | I                   | {B<br>C<br>D     | 533<br>526<br>525 |
| 14          |                                                                         | —NHSO <sub>2</sub><br>C <sub>6</sub> H <sub>5</sub>                                                            | IV                  | B                | 530               |
| 15          |                                                                         | —NHCO—<br>C <sub>6</sub> H <sub>11</sub>                                                                       | IV                  | B                | 528               |
| 16          |                                                                         | —N—<br>C <sub>6</sub> H <sub>11</sub><br>CO                                                                    | IV                  | B                | 529               |
| 17          |                                                                         | —NHCOOC <sub>6</sub> H <sub>4</sub> OMe <sub>2</sub>                                                           | II                  | B                | 443               |
| 18          |                                                                         | —N—<br>C <sub>6</sub> H <sub>11</sub><br>COCH <sub>2</sub> CH <sub>3</sub>                                     | II                  | D                | 432               |
| 19          |                                                                         | —N—<br>C <sub>6</sub> H <sub>11</sub><br>COCH(CH <sub>3</sub> ) <sub>2</sub>                                   | II                  | D                | 430               |

| Exam p<br>No. | Structure of color coupler R—NHCOCH—CH—COOH |                |                | Formu-<br>lation<br>Process | Devel-<br>oping<br>Agent | $\lambda$ max. |
|---------------|---------------------------------------------|----------------|----------------|-----------------------------|--------------------------|----------------|
|               | R                                           | R <sub>1</sub> | R <sub>2</sub> |                             |                          |                |
| 20            |                                             |                |                | II                          | D                        | 425            |
| 21            |                                             |                |                | II                          | D                        | 420            |
| 22            |                                             |                |                | II                          | D                        | 430            |
| 23            |                                             |                |                | II                          | D                        | 422            |
| 24            |                                             |                |                | II                          | D                        | 429            |
| 25            |                                             |                |                | II                          | {B<br>C                  | 440<br>446     |
| 26            |                                             |                |                | III                         | {B<br>C                  | 665<br>645     |
| 27            |                                             |                |                | III                         | C                        | 647            |
| 28            |                                             |                |                | III                         | C                        | 650            |
| 29            |                                             |                |                | III                         | {C<br>D                  | 664<br>654     |
| 30            |                                             |                |                | III                         | {C<br>D                  | 663<br>653     |

| Example No. | Structure of color coupler R—NHCOCH—CH—COOH |                                                                                         | Formulation Process | Developing Agent | $\lambda$ max. |
|-------------|---------------------------------------------|-----------------------------------------------------------------------------------------|---------------------|------------------|----------------|
|             | R                                           | R <sub>1</sub> R <sub>2</sub>                                                           |                     |                  |                |
| 31.....     |                                             | —NHCOOC <sub>17</sub> H <sub>35</sub>                                                   | III                 | B<br>C           | 668<br>673     |
| 32.....     |                                             | —NHCOOC <sub>17</sub> H <sub>35</sub> .....                                             | III                 | C                | 644            |
| 33.....     |                                             | —N<br> <br>nC <sub>18</sub> H <sub>37</sub><br> <br>COCH(CH <sub>3</sub> ) <sub>2</sub> | III                 | C                | 644            |
| 34.....     |                                             | —NHCOOC <sub>17</sub> H <sub>35</sub> .....                                             | III                 | B                | 645            |

*Example 35*

To 200 parts of a gelatino-silver bromide emulsion there are added 50 parts of a 5% aqueous solution of the sodium salt of 4'-stearoylaminobenzoylacet-3:5-dicarboxyanilide. The blue sensitive emulsion so obtained is coated on a paper base and the coated layer dried. A 3% aqueous solution of gelatin is then coated on top of the blue sensitive layer to form a gelatin separation layer. A green sensitive emulsion obtained as described in Example 1 is then coated on top of the gelatin separation layer. A gelatin separation layer is then coated on top of the green sensitive emulsion layer. A red sensitive emulsion comprising 200 parts of a red sensitive gelatino-silver chlorobromide emulsion and 50 parts of a 5% aqueous solution of the sodium salt of 1-hydroxy-4-sulpho-2-naphtho-N-octadecylamide is then coated on top of the gelatin separation layer.

The multilayer color photographic paper so obtained is exposed to the light from a color negative, developed in a color developer containing 4-amino-3-methyl-N-diethyl-aniline, bleached and fixed. A color print is obtained.

*Example 36*

In place of the green sensitive emulsion used in Example 35 there is used a green sensitive emulsion obtained by adding 50 parts of a 5% aqueous solution of the potassium salt of the coupler of Example 9 to 200 parts of a green sensitive gelatino-silver chlorobromide emulsion.

When the multilayer color photographic paper so obtained is exposed to the light from a color negative, developed in a color developer containing 4-amino-3-methyl-N-diethyl-aniline, bleached and fixed, a color print is obtained.

What I claim is:

1. A process for the production of a color photograph image which comprises subjecting reducible silver salt image to development by means of an aromatic primary amino-color developing agent in the presence of a color coupler of the formula



wherein Y is selected from the group consisting of hydrogen, an alkali metal and an amine group, where R is selected from the group consisting of (a) a benzyl aceto acetanilide having the structural formula:



wherein R<sub>3</sub> is selected from the group consisting of phenyl and alkoxy phenyl and R<sub>4</sub> is selected from the group consisting of phenyl, alkoxy phenyl and alkyl amino phenyl, (b) a cyanoacetyl aniline having the structural formula



wherein R<sub>5</sub> and R<sub>6</sub> are selected from the group consisting of hydrogen and lower alkyl, (c) an amino 2-pyrazoline-5-one having the structural formula



wherein R<sub>7</sub> is selected from the group consisting of



and



and R<sub>8</sub> is a phenyl group, (d) a phenol having the structural formula





at least one layer of a light sensitive silver halide emulsion, containing dispersed therein a color coupler of the formula



5

where  $Y$  is selected from the group consisting of hydrogen, an alkali metal and an amine group, where  $R$  is selected from the group consisting of (a) a benzyl aceto acetanilide having the structural formula:



wherein  $R_3$  is selected from the group consisting of phenyl and alkoxy phenyl and  $R_4$  is selected from the group consisting of phenyl, alkoxy phenyl and alkyl amino phenyl, (b) a cyanoacetylaniline having the structural formula



15

wherein  $R_5$  and  $R_6$  are selected from the group consisting of hydrogen and lower alkyl, (c) an amino 2-pyrazoline-5-one having the structural formula



wherein  $R_7$  is selected from the group consisting of



and



and  $R_8$  is a phenyl group, (d) a phenol having the structural formula



wherein  $R_9$  is selected from the group consisting of



and  $R_{10}$  is selected from the group consisting of hydrogen, halogen, alkyl and alkoxy, and (e) a 1-naphthol selected from the group consisting of the structural formulae



15

20

wherein  $R_{11}$  is selected from the group consisting of  $-NH$  and  $-CO-NH-R_{13}-NH-$ , wherein  $R_{13}$  is selected from the group consisting of alkylene and arylene, and  $R_{12}$  is selected from the group consisting of hydrogen and halogen, and where either one of  $R_1$  and  $R_2$  is a hydrogen atom and the other is a radical selected from the group consisting of

30



35

wherein  $R_{14}$  is an acyl radical selected from the group consisting of alkanyl having 1 to 18 carbon atoms, phenoyl, alkylsulfonyl, alkenylsulfonyl and alkylphenylsulfonyl,  $R_{15}$  is selected from the group consisting of hydrogen, an alkyl group, a cycloalkyl group, an aralkyl group and an aryl group and  $Z$  is selected from the group consisting of ethylene, phenylene and tetrahydrophenylene.

14. A photographic element according to claim 13 wherein  $R_{15}$  is an alkyl having at least 12 carbon atoms.

40

45

References Cited in the file of this patent

UNITED STATES PATENTS

2,964,402 Jennen et al. ----- Dec. 13, 1960